

July 5, 1966

E. A. BRANDES ET AL

3,259,560

PROCESS FOR THE ELECTROLYTIC PRODUCTION OF  
CHROMIUM OF A HIGH DEGREE OF PURITY  
Filed July 20, 1962



Inventors  
Eric Adolph Brandes  
James Abraham Whitaker  
By  
Albert J. Jacks  
Attorney

## 1

3,259,560

**PROCESS FOR THE ELECTROLYTIC PRODUCTION OF CHROMIUM OF A HIGH DEGREE OF PURITY**  
 Eric A. Brandes, Chalfont St. Peter, and James A. Whittaker, Slough, England, assignors to National Research Development Corporation, London, England, a corporation of Great Britain

Filed July 20, 1962, Ser. No. 211,246  
 Claims priority, application Great Britain, July 26, 1961,

27,061/61  
 2 Claims. (Cl. 204—105)

This invention relates to a process for the electrolytic deposition of chromium of a high degree of purity.

It has heretofore been proposed in the electrolytic deposition or electro-winning of chromium to use fluoride baths containing 250 g./litre  $\text{CrO}_3$  and 5 g./litre HF and lead alloy anodes, the most favoured lead alloys being those with a tin constituent, for example  $\text{Pb}/7\%$  Sn. The chromium obtained using such anodes has been contaminated in some degree by tin and could not be used in circumstances requiring chromium of a high degree of purity. Pure lead is not satisfactory in that it is attacked by the electrolyte, particularly when this operates at high temperature.

To obtain chromium free from nitrogen and oxygen it is necessary to use the electrolyte at high temperature, preferably as nearly as practicable to the boiling point of the electrolyte, to reduce the solubility of these gases in aqueous solution. The fluoride bath has the advantage that its efficiency increases with increase in temperature. Other baths used for the production of electrodeposited chromium, notably the sulphate bath containing 250 g./litre  $\text{CrO}_3$  and a

$$\frac{\text{CrO}_3}{\text{SO}_4} = \frac{100}{1}$$

decrease in efficiency as the temperature is varied.

An object of the present invention is a process of winning chromium of a high degree of purity which comprises producing same electrolytically in a fluoride bath

| Run No. | 58 litres of solution in a 60 litre polythene tank                | Cathode Current Density, amps./ft. <sup>2</sup> | Duration of Run in Hours | Bath Temp., °C. | Cathode Current Efficiency, percent |    |
|---------|-------------------------------------------------------------------|-------------------------------------------------|--------------------------|-----------------|-------------------------------------|----|
|         |                                                                   |                                                 |                          |                 | 460                                 | 30 |
| 1.....  | New solution uncoated palladium anode. No lead additions to bath. | 460                                             | 24                       | 90              |                                     | 30 |
| 2.....  | do                                                                | 460                                             | 24                       | 90              |                                     | 28 |
| 3.....  | do                                                                | 460                                             | 24                       | 90              |                                     | 25 |
| 4.....  | do                                                                | 460                                             | 24                       | 90              |                                     | 15 |
| 5.....  | do                                                                | 460                                             | 24                       | 90              |                                     | 14 |
| 6.....  | do                                                                | 460                                             | 24                       | 90              |                                     | 13 |

TABLE 2  
 [Solution composition 250 g./l.  $\text{CrO}_3$ ; 5 g./l. HF.]

| Run No. | 9 litres of the solution in a 10 litre PTFE beaker                | Cathode Current Density, amps./ft. <sup>2</sup> | Duration of Run in Hours | Bath Temp., °C. | Cathode Current Efficiency, Percent |
|---------|-------------------------------------------------------------------|-------------------------------------------------|--------------------------|-----------------|-------------------------------------|
| 1.....  | New solution uncoated palladium anode. No lead additions to bath. | 460                                             | 6                        | 80              | 29                                  |
| 2.....  | do                                                                | 520                                             | 6                        | 90              | 23                                  |
| 3.....  | do                                                                | 410                                             | 6                        | 95              | 15                                  |

It will be apparent from Tables 1 and 2 that when a new solution is used with no lead either on the anode or in the bath, the initial results are quite good but there is a rapid falling off in efficiency in subsequent runs.

The following three tables are exemplary of a series of runs made with apparatus according to the present invention as exemplified in the accompanying drawing, and utilizing the method according to the present invention, in the electrolytic production of chromium of a high degree of purity from a solution of chromic anhydride ( $\text{CrO}_3$ ) in hydrofluoric acid (HF). As regards Tables 3 and 4, the high density polythene tank of the apparatus shown in the drawing is replaced by a PTFE beaker.

normal for the analar grade of chromic acid, as it has been found that the nitrogen content of the electrolyte, particularly if present as a nitrate or nitrite is reflected in the nitrogen content of the chromium deposited on the cathode, and in the continuing efficiency of the process after a number of runs. The nitrogen content in the deposited chromium was found to be about 10 p.p.m. with chromic acid of 12 p.p.m. nitrogen content.

10 The pure electrodeposited chromium deposited in the manner described may be used as a decorative or protective coating or after removal from the cathode, may be used to produce chromium based alloys for use at high temperatures or stainless steel or other ferrous alloys having extremely low carbon, oxygen and nitrogen con-

TABLE 3  
[Solution composition 250 g./l.  $\text{CrO}_3$ ; 5 g./l. HF.]

| Run No. | 9 litres of the solution in a 10 litre PTFE beaker                       | Cathode Current Density, amps./ft. <sup>2</sup> | Duration of Run in Hours | Bath Temp., °C. | Cathode Current Efficiency, Percent |
|---------|--------------------------------------------------------------------------|-------------------------------------------------|--------------------------|-----------------|-------------------------------------|
| 1.....  | Palladium anode. Bath saturated with lead chromate ( $\text{PbCrO}_4$ ). | 435                                             | 4.25                     | 95              | 31                                  |
| 2.....  | do.....                                                                  | 435                                             | 6                        | 95              | 32                                  |
| 3.....  | do.....                                                                  | 435                                             | 5.5                      | 95              | 27                                  |
| 4.....  | do.....                                                                  | 460                                             | 6                        | 95              | 22                                  |

TABLE 4  
[Solution composition 250 g./l.  $\text{CrO}_3$ ; 5 g./l. HF.]

| Run No. | 9 litres of the solution in a 10 litre PTFE beaker                                                                                                                     | Cathode Current Density, amps./ft. <sup>2</sup> | Duration of Run in Hours | Bath Temp., °C. | Cathode Current Efficiency, Percent |
|---------|------------------------------------------------------------------------------------------------------------------------------------------------------------------------|-------------------------------------------------|--------------------------|-----------------|-------------------------------------|
| 1.....  | Palladium anode. Bath saturated with $\text{PbCrO}_4$ and anode coated with $\text{PbO}_2$ by anodic treatment in saturated lead fluoride ( $\text{PbF}_2$ ) solution. | 460                                             | 6                        | 95              | 26                                  |
| 2.....  | do.....                                                                                                                                                                | 460                                             | 5.75                     | 95              | 30                                  |
| 3.....  | do.....                                                                                                                                                                | 460                                             | 5                        | 95              | 30                                  |
| 4.....  | do.....                                                                                                                                                                | 460                                             | 5.5                      | 95              | 28                                  |
| 5.....  | do.....                                                                                                                                                                | 460                                             | 5.75                     | 95              | 29                                  |
| 6.....  | do.....                                                                                                                                                                | 460                                             | 5.5                      | 95              | 28                                  |

TABLE 5  
Solution composition 250 g./l.  $\text{CrO}_3$ ; 5 g./l. HF.]

| Run No. | 55 litres of solution in a high-density polythene tank                                                                                                 | Cathode Current Density, amps./ft. <sup>2</sup> | Duration of Run in Hours | Bath Temp., °C. | Cathode Current Efficiency, percent |
|---------|--------------------------------------------------------------------------------------------------------------------------------------------------------|-------------------------------------------------|--------------------------|-----------------|-------------------------------------|
| 1.....  | Palladium anode. Bath saturated with $\text{PbCrO}_4$ and $\text{PbO}_2$ formed on the anode by anodic treatment in saturated $\text{PbF}_2$ solution. | 460                                             | 24                       | 95              | 34                                  |
| 2.....  | do.....                                                                                                                                                | 460                                             | 24                       | 95              | 38                                  |
| 3.....  | do.....                                                                                                                                                | 460                                             | 24                       | 95              | 37                                  |
| 4.....  | do.....                                                                                                                                                | 460                                             | 24                       | 95              | 37                                  |
| 5.....  | do.....                                                                                                                                                | 460                                             | 24                       | 95              | 37                                  |
| 6.....  | do.....                                                                                                                                                | 460                                             | 24                       | 95              | 36                                  |
| 7.....  | do.....                                                                                                                                                | 460                                             | 24                       | 95              | 38                                  |

Spectrographic examination of the chromium yield in all cases failed to show the presence of any lead in the chromium.

It will be manifest from a comparison of Tables 3 to 5 that best results can be expected when lead is present both in the bath and on the anode. It will also be apparent from Tables 1 and 2 that the efficiency of the bath increases with greater bulk of electrolyte and a ratio of volume of electrolyte in litres to area of cathode in square inches of not less than 0.6 has been found to be necessary for efficient operation.

It is preferred to make up the bath with chromic acid having a low nitrogen content e.g. chromic acid having a nitrogen content of 12 p.p.m. instead of the 40 p.p.m.

70 75 contents. Examples of such alloys are alloys with iron containing up to 40% chromium.

We claim:

1. In an electrolytic process for the production of high purity chromium from a fluoride bath of dissolved chromic acid low in nitrogen the improvements comprising:
  - (a) carrying out the electrolysis at a temperature of at least 85° C.,
  - (b) carrying out the electrolysis with an anode of material selected from the group consisting of platinum, platinum alloys, palladium and palladium alloys,
  - (c) carrying out the electrolysis with lead chromate present in the bath, and
  - (d) maintaining a coating of lead dioxide on said anode material.

2. In an electrolytic process, according to claim 1, the further improvements comprising:

- (a) carrying out the electrolysis at a cathode current density of from 435 to 460 amperes per square foot and
- (b) carrying out the electrolysis in a bath having a ratio of volume in litres of said bath to the area of cathode in square inches of at least 0.6.

**References Cited by the Examiner**

**UNITED STATES PATENTS**

|           |        |            |       |        |    |
|-----------|--------|------------|-------|--------|----|
| 1,544,451 | 6/1925 | Hambuechen | ----- | 204—51 | 10 |
| 2,307,551 | 1/1943 | Triska     | ----- | 204—51 |    |
| 2,704,273 | 3/1955 | Yoshida    | ----- | 204—51 | 15 |

|           |         |                |       |         |
|-----------|---------|----------------|-------|---------|
| 2,766,202 | 10/1956 | Estes          | ----- | 204—242 |
| 2,787,588 | 4/1957  | Stareck et al. | ----- | 204—51  |
| 2,969,314 | 1/1961  | Coxe           | ----- | 204—242 |

**FOREIGN PATENTS**

|   |         |         |         |
|---|---------|---------|---------|
| 5 | 586,846 | 11/1959 | Canada. |
|---|---------|---------|---------|

**OTHER REFERENCES**

Morisset, Paul et al.: "Chromium Plating," Rober Draper Ltd., page 207, 1954.

JOHN H. MACK, *Primary Examiner*.

JOHN R. SPECK, MURRAY TILLMAN, *Examiners*.

G. KAPLAN, *Assistant Examiner*.